

# UNITED STATES PATENT OFFICE.

ROBERT JOHNSON TILFORD, OF LOUISVILLE, KENTUCKY.

## PROCESS OF UNITING METALS

SPECIFICATION forming part of Letters Patent No. 424,379, dated March 25, 1890.

Application filed November 1, 1889. Serial No. 328,956. (No specimens.)

To all whom it may concern:

Be it known that I, ROBERT JOHNSON TILFORD, a citizen of the United States, residing at Louisville, in the county of Jefferson and State of Kentucky, have invented a certain new and useful Process for Uniting Metals; and I do declare the following to be a full, clear, and exact description of the invention, such as will enable others skilled in the art to which it appertains to make and use the same.

My invention relates to an improved process of welding iron to steel or steel to steel, in both cases the sections to be united having different percentages of carbon.

15 Heretofore many attempts to perfectly weld such metals have been attempted, but in so far as I am aware without success. The most common method known to me consists in arranging steel and iron in a pile, subjecting 20 said pile to a welding heat, and thereafter subjecting it to "rolling, hydraulic pressure, hammering, or all." The product obtained by such methods is suitable for some purposes; but, generally speaking, is commercially unsatisfactory by reason of the fact that when 25 subjected to shocks or concussions above a certain degree it has its coherency destroyed and the iron split or separated from the steel, the result being that the product is fractured.

30 By my improved process I avoid the objections attendant upon previous methods, and I am enabled to produce a compound product in which the welding of the two metals to be united is so thoroughly effected that their allied faces become practically obliterated and the metal homogeneous therat.

In conducting welding operations in accordance with my said process set forth herein I have found that important and valuable results are also obtained by employing a steel previously treated in accordance with the Letters Patent No. 397,476, issued February 5, 1889, to myself and one H. M. Redemann, to which reference may be had for a more 45 complete understanding of the said process and the condition of the product before and after such treatment. By reference to said patent it will be found that the improved process set forth and claimed therein relates to subjecting Bessemer and other low grades of steel heated to such heat as may be desired to a previously-prepared liquid bath of

such character that the contact of metal and liquid bath induces hydrocarbon gases, which are absorbed or taken up by the metal, the latter being permitted to remain in such bath at pleasure or until substantially cool or until such reduction of heat is made that it will no longer take up hydrocarbon gases. The results consequent upon such patented process are stated to be inexpensive production of a higher grade of steel, minimum degree of labor involved therein, and the procurement of a product having a molecular change from a coarse grain to a fine grain or silky fracture to increase tensile strength, elasticity, toughness, and ductility, and to greatly increase the carbon. The principal elements of the bath mentioned are glycerine and water in the proportion of three ounces of glycerine to one-half gallon of water. To such elements may be added spirits of niter, aqua-ammonia, chloride of ammonium, sulphate of zinc, sulphate of alumina, and ammonia. The steps and agents involved in said patented process have been here detailed, for when the product thereof is used in the process forming the subject-matter of the present application such steps and agents constitute a sub-process and will be directly related thereto. It is further proper to here state that one of the advantages secured for steel treated by said patented process is its capacity for resisting impairment by reheating, if such reheating is conducted at any temperature representing a degree of heat below what would be required to effect in part or wholly the destruction of the steel qualities of the article.

In carrying out the present process in the event of the union of iron to steel two or more furnaces are employed, and the iron, which is the wrought-iron of commerce, is heated in one furnace to a high degree, equivalent to a dazzling white or just below its melting-point. The steel to be united therewith, heated in a separate furnace to a degree approaching incipient redness, is placed in contact with the iron, the surfaces, if desired, having been previously fluxed or otherwise prepared to contribute to the union of the two metals. The relatively-arranged iron and steel are then placed in either of the two furnaces mentioned or in a separate furnace,

and are then gradually heated until the steel assumes substantially a bright-red color, at which period the metal is either hammered or rolled, or both, to condense and reduce it 5 completely into a compound product, in which the iron and steel exist in a perfect union or weld. By heating the iron to a degree so much higher than the steel, contact with the steel will, by reason of its greater heat, begin

- 10 to withdraw a part of the carbon of the steel, which becomes incorporated in the said iron or portion of said iron at about the instant the two metals are brought in contact, the union finally becoming so complete that the 15 steel merges into the iron regularly and evenly, and thereby avoids the weakness that would exist were the junction of the two more sharply defined.

It will be understood that by heating the 20 iron to the high degree mentioned and the steel to an incipient redness, and then arranging them relative to each other, it will not be necessary in the succeeding operations required to reduce and complete the compound 25 article to heat the external faces of the steel to an excessive extent in order to raise the covered face or portion adjacent to the iron to a welding degree. By such practice I am enabled to avoid the burning out or deterioration 30 of the steel, which generally attends the practice where the metals are arranged in a pile before heating.

I do not wish to be understood as limiting myself in the present process to the welding 35 with iron or low-grade steel of a steel produced by said patented process previously mentioned, as it will be quite obvious that other kinds of steels of varying quality or grade may be successfully welded to each 40 other or to iron.

In giving the steel a preliminary heating, where considered necessary, of comparative low degree, before arranging it relative to the iron, undue or sudden expansion, when 45 brought into proximity to the highly-heated iron, is avoided, and hence liability to cracking or fracture is avoided.

As before stated, the process is applicable for securing a regular and complete welding 50 of high and low grade steel or of steel generally with iron.

In the within description, when iron is mentioned the wrought-iron of commerce is referred to, and when such iron is to be united

with steel it will be with either of the qualities known as "high" and "low" grade cast-steel 55 of the Bessemer production. When steel is to be united to steel, the description contemplates two independent steel sections having pronounced differences of carbon, thus constituting the same relative relation and character 60 that exists between wrought-iron and steel.

I claim—

1. The improved step in the art of uniting 65 wrought-iron and steel or steel to steel having different percentages of carbon, the same consisting in heating the metal lowest in carbon to a degree equivalent to white heat, heating the metal highest in carbon to an incipient 70 red heat, and thereafter placing the two differently-heated metals in contact, substantially as set forth.

2. The process of uniting wrought-iron and steel or steel to steel having different percentages of carbon, the same consisting in heating the metal lowest in carbon to a white heat, heating the metal highest in carbon to an incipient red heat, placing both metals in 75 contact in a furnace and heating to a welding 80 heat, and finally subjecting to a further welding action, substantially as set forth.

3. The process of uniting steel with a metal having a comparative lower percentage of carbon, consisting in first subjecting steel at 85 a white heat to the action of a liquid bath evolving hydrocarbon gases, heating the metal low in carbon to a high temperature, and then arranging the steel relative thereto, and finally uniting, substantially as shown and 90 set forth.

4. The process of uniting steel with a metal having a comparative low percentage of carbon, consisting in first subjecting steel at a white heat to the action of a liquid bath 95 evolving hydrocarbon gases until said steel reaches the limit of its absorption, then heating the metal low in carbon to a high temperature, moderately heating the steel, relatively arranging it with respect to the highly-heated 100 metal, and finally uniting, substantially as shown and set forth.

In testimony whereof I affix my signature in presence of two witnesses.

ROBERT JOHNSON TILFORD.

Witnesses:

DARWIN W. JOHNSON,

DAVID BARTLEY.